

## UNITED STATES PATENT OFFICE

WALTER GLAESER, OF BROOKLYN, NEW YORK, ASSIGNOR TO GLAESER RESEARCH CORPORATION, OF NEW YORK, N. Y., A CORPORATION OF NEW YORK

## METHOD OF PRODUCING MERCURY

No Drawing.

Application filed November 14, 1924. Serial No. 749,999.

The present invention relates to a new and improved method of producing mercury, and is particularly directed to a method of extracting mercury from cinnabar ore in a wet way and without the necessity for subliming the ore as is the case in the method now in general use. My improved process is very much more economical than that now in use and is capable of effecting a recovery of better than 90 per cent of the total amount of mercury in the ore, while at the same time ores of any amount of mercury content can be economically treated. To the accomplishment of the foregoing and related ends, said invention, then, consists of the means hereinafter fully described and particularly pointed out in the claims.

The following description sets forth in detail one approved method of carrying out the invention, such disclosed mode, however, constituting but one of the various ways in which the principle of the invention may be used.

In my improved process cinnabar ore (mercuric sulphide) is crushed and pulverized until it will pass a relatively fine screen, say from 80 to 150 mesh, the fineness of the crushed ore affecting the speed and completeness of reactions in the further steps of the process. This finely crushed cinnabar ore is then mixed with a sufficient amount of water to form a thin paste, and a reducing gas, preferably nascent hydrogen, is introduced in any suitable way. One convenient manner involves adding to the paste a hydroxide of an alkali metal or alkaline earth metal in excess and a metal reactive therewith to produce hydrogen, for instance finely divided metal in the form of filings or turnings if desired, such as aluminum, zinc, iron, brass, copper, etc. On employing aluminum proper steps must be taken to prevent the too rapid formation and loss of nascent hydrogen, which also causes the alu-

minum to be consumed to an excessive degree. Zinc, brass, an alloy of aluminum or aluminum are the metals which I prefer to use.

This composition is then heated to a temperature of from 50 to 90 degrees C. for substantially one hour. The reactions will vary in speed with the temperature, but the mixture should be warmed to a certain extent in order to hasten the reaction.

The reactions which take place are, first, a reaction between the hydroxide and the zinc to form a zincate, or the aluminum to form an aluminate, liberating nascent hydrogen. This nascent hydrogen then attacks the red cinnabar ore, liberating metallic mercury and hydrogen sulphide. The hydrogen sulphide combines with the zincate to form zinc sulphide and the original alkaline hydroxide is recovered. The mercury then mechanically combines with the metal which is present, such as zinc, to form a mercury zinc amalgam. The complete series of reactions which it is assumed take place in the mixture are as follows:

1.  $Zn + 2NaOH = Zn(ONa)_2 + H_2$
- 1<sup>a</sup>.  $2Al + 6NaOH = Al_2(ONa)_6 + 3H_2$
2.  $Red. HgS + H_2 = Hg + H_2S$
3.  $Zn(ONa)_2 + H_2S = ZnS + 2NaOH$
- 3<sup>a</sup>.  $Al_2(ONa)_6 + 3H_2S = Al_2(OH)_6 + 3Na_2S$
4.  $Hg + Zn = Hg.Zn$  (zinc amalgam)

It is possible that after the liberation of the mercury a further reaction takes place which may be represented as follows:

5.  $Red. HgS$  (2 molecules) +  $H_2 =$   
Black  $HgS + Hg + H_2S$
6.  $NaOH + H_2S = NaSH + H_2O$  or  
 $3Na_2S$  (from 3<sup>a</sup>) +  $3H_2S = 6NaSH$

It is probable that a further reaction takes place in the presence of caustic soda between the black sulphide of mercury produced under reaction No. 5 and some sodium sulphhydrate which has been formed under reaction

No. 6 for it is found that temporarily some soluble mercury compound appears in solution. The reactions covering this phase may be represented as follows:—



This double sulphide of mercury and sodium is soluble in water; it reacts with a metal like zinc or aluminum in the following manner:



It is found that the mixture after the initial reaction turns black when copper instead of zinc or aluminum is used, and it is presumed that this is caused by the formation of some black sulphide of copper. A similar black discoloration appears on using zinc or aluminum if the original ore contains an appreciable amount of iron compounds as impurity, causing formation of black sulphide of iron. If a large amount of iron compounds or other sulphur binding compounds are present in the ore it may become necessary to supply an amount of soluble sulphide to the mixture sufficient to take care of such compounds.

After freeing the mercury from the cinnabar ore and converting it into a mercury zinc amalgam the latter is removed from the solution, is washed, and then distilled above 360° C. in order to drive off the mercury, which is then condensed, the zinc being in this way entirely purified from the mercury and is usable over again in the process.

The present process is carried out entirely in an aqueous solution, is simple and quite inexpensive, and is relatively fast and gives, particularly if the solution is maintained between the temperatures given above and is agitated during the reaction, a recovery of better than 90 per cent. of the original mercury content of the ore.

The decomposition of the cinnabar may also be effected by agitating the powdered ore with warm water and a metal or a metal couple such as a zinc-copper couple or a copper aluminum couple or any other aluminum alloy in the presence of a trace of an acid. The metal or the metal couples decompose water under these conditions, releasing hydrogen which desulphurizes the ore, freeing the mercury which is then acted upon and recovered as already described.

Other modes of applying the principle of my invention may be employed instead of the one explained, change being made as regards the process herein disclosed, provided the step or steps stated by any of the following claims or the equivalent of such stated step or steps be employed.

I therefore particularly point out and distinctly claim as my invention:—

1. A method of extracting mercury from cinnabar ore, which comprises liberating the mercury by treating the finely divided ore in the presence of water with a reducing gas reactive with such ore. 70

2. A method of extracting mercury from cinnabar ore, which comprises subjecting the finely divided ore to a reducing agent in the presence of water and a metal capable of forming an amalgam with the mercury. 75

3. In a method of extracting mercury from cinnabar ore, the steps which consist in reacting upon finely divided cinnabar ore with a nascent gas capable of displacing mercury from combination, in the presence of water and a finely divided metal, and removing and distilling the mercury amalgam there formed. 80

4. In a method of extracting mercury from cinnabar ore, the steps which consist in agitating the finely ground ore in water, while causing liberation of hydrogen from the water. 85

5. In a method of extracting mercury from cinnabar ore, the steps which consist in agitating finely ground cinnabar ore with water in the presence of a metal couple to liberate hydrogen from the water, amalgamating the mercury, and then removing and distilling the mercury amalgam thus formed. 90

6. A method of extracting mercury from cinnabar ore, which comprises liberating the mercury by treating the ore in the presence of water with a reducing gas reactive with such ore. 95

7. In a method of extracting mercury from cinnabar ore, the steps which consist in agitating the ore in water, while causing liberation of hydrogen from the water. 100

Signed by me, this 20th day of September, 1924.

WALTER GLAESER.

110

115

120

125

130